

# UNITED STATES PATENT OFFICE.

ANTON LEDERER, OF ATZGERSDORF, NEAR VIENNA, AUSTRIA-HUNGARY.

## SUPPORT FOR METALLIC GLOW-FILAMENTS.

1,203,635.

Specification of Letters Patent.

Patented Nov. 7, 1916.

No Drawing.

Application filed September 18, 1906. Serial No. 335,152.

*To all whom it may concern:*

Be it known that I, ANTON LEDERER, a subject of the Empire of Austria-Hungary, residing at No. 83, Atzgersdorf, near Vienna, 5 in the Province of Lower Austria, Austria-Hungary, have invented certain new and useful Improvements in Supports for Metallic Glow-Filaments, of which the following is a specification.

10 My invention relates to improvements in metallic supports for metallic glow filaments for electric incandescent lamps, and it has for its object to provide metallic supports of such a construction and composition 15 that they will prevent bulging of the filament when the latter expands in consequence of its being heated by the electric current.

20 The necessity of supporting metallic glow filaments in electric incandescent lamps has been proved long since. Metallic filaments, however, do not allow the use of metallic supports, as is customary with electric incandescent lamps having carbon filaments. 25 When supports of platinum or other bare (non-oxidized) metals are used, it has been observed that the filaments may become fritted to the support. This fact is of no disturbing influence with lamps that are continuously in use, that is to say, that are not 30 frequently cut out of circuit. However, if a lamp is repeatedly and often cut in and out of circuit, as is usually the case, it is observed that the filament surrounded and 35 held by the support visibly bulges in the part of its length adjacent to the point of contact with the support. This bulging may cause short circuiting and other disagreeable disturbances. This phenomenon may

40 be explained as follows: When the filament becomes fritted to the support and then strongly contracts after having been cut out of circuit, there is formed at the place of fritting a kind of angle or knot which prevents the free and unhindered expansion of 45 the filament. With the successive operations of the lamp, new enlargements or knots are liable to be formed at other points along the length of filament so that the filament 50 cannot readily slide through the support and it is thus caused to bulge outward.

This present invention has for its object

to prevent deformations of the glow filament such as those above described, and still to allow the use of metallic supports, 55 by coating the supports with an extremely thin layer of a compound of the metal used for the support, preferably with an oxid of such metal. The layer of oxid being extremely thin, the support formed according 60 to the present invention retains its power of conducting heat, so that, on the one hand, no reduction of the oxid can take place and, on the other hand, the glow filament is prevented from fritting to the metallic support 65 by the protecting coating of oxid.

The supporting wire may be easily and conveniently provided with a coating of oxid by passing it through an oxidizing flame. Nickel is an excellent metal for use 70 as the oxidized filament support, but I do not wish to be restricted to the use of nickel, since any metal which is sufficiently refractory and which can be covered with a protective coating of one of its compounds is 75 suitable for my use. I am aware that filament supports have heretofore been made having filament-supporting loops or rings of refractory oxids attached to their ends. My filament supports are distinguished 80 from these by the fact that my protective coatings are composed of compounds of the supporting metals themselves, and by the fact that the coatings do not extend beyond the ends of the supports, and are thus 85 interposed between the filaments and the supporting wire. Since the filaments are separated from the metal wire only by the thin coating, heat is quickly conducted away from the filament, and harmful localization 90 of heat is thereby avoided.

What I claim as my invention and desire to secure by Letters Patent is:

1. In a metal filament incandescent lamp, a support for the metallic filament consisting of a metal wire, coated with an oxygen compound of the metal of the said wire, which coating does not extend beyond the end of the support and is thus interposed between the filament and the said metal wire. 100
2. In an electric lamp, the combination of a metallic filament and a support for the said filament consisting of a nickel wire, coated with oxid of nickel; said covering

being thus interposed between the said filament and the nickel wire.

3. As a support for incandescent metal, a wire of high refractability consisting of a nickel wire coated with an oxid of nickel.

4. A shield for the support of an incandescent metal body, consisting of a coating of an oxid of the metal out of which said support is made, the said coating being thus

interposed between the incandescent metal body and the metal of the support.

In witness whereof I have hereunto set my hand in presence of two witnesses.

ANTON LEDERER.

Witnesses:

JOHANN LUSCH,  
ALVESTO S. HOGUE.